

## UNITED STATES PATENT OFFICE

RALPH L. BINNEY, OF TOLEDO, OHIO, ASSIGNOR TO THE BINNEY CASTINGS COMPANY, OF TOLEDO, OHIO, A CORPORATION OF OHIO

## FERROUS ALLOY

No Drawing.

Application filed May 20, 1931. Serial No. 538,875.

This invention relates to a ferrous alloy having great resistance to deterioration when subjected alternately to elevated and low temperatures, and also having a high resistance to scaling, cracking, and warping at high temperatures.

The alloy, in addition to iron and carbon contains aluminum, silicon, chromium, and vanadium.

10 The alloy has a tensile strength of approximately 45000 pounds per square inch, which is about twice that of ordinary cast iron. Its hardness is also about twice that of ordinary cast iron, the alloy having a Brinell hardness of about 325. Although the alloy has a hardness and strength approximately double that of ordinary cast iron, its machinability does not differ greatly from ordinary cast iron, and for this reason it can be used where cast 15 iron has been employed formerly, but where it is desired that the alloy be able to withstand alternate heating and cooling and also withstand high temperatures without substantial deformation. Its expansion upon 20 heating is slightly less than cast iron and it has less permanent growth.

The alloy is exceedingly fine grained and takes a better polish than cast iron, due to its denser nature. Softening does not occur 25 at temperatures above 1300° F., which temperature is higher than is necessary to produce softening in ordinary cast iron. Even at a temperature of 1500° F., the hardness of the alloy is about 255 Brinell. Due to the 30 fact that the alloy retains its hardness and strength at temperatures of 1500° F. or above, the alloy is unusually well suited for making glass molds where these properties enable the material to retain edges that do not break 35 off or pean down. The marked ability of the alloy to resist tempering or softening at elevated temperatures makes it extremely valuable for use under conditions where strength 40 and hardness are required while an alloy is very hot.

The alloy is particularly adapted for molds for forming glass and parts of glass equipment coming in contact with molten glass or subjected to high temperatures, furnace 45 equipment, valves for internal combustion

engines, molds for die-casting machines, and for any uses requiring a metal having greater strength or hardness than cast iron, or where the article must withstand high temperatures or alternate heating and cooling without substantial scaling, cracking, warping or deformation.

The ferrous alloy having these properties contains carbon about 2.5% to 3.5%, aluminum about 2.0% to 3.5%, silicon about 2.0% to 3.5%, chromium about 2.0% to 3.5%, and about .10% to .50% of vanadium. The alloy may also contain sulphur, phosphorous and manganese in small amounts as impurities, but for best results neither the sulphur 60 nor the phosphorus should exceed .04%, and the manganese should not exceed .20%.

I also have found that when the aluminium, silicon, and chromium contents of the alloy are each about 3%, the desirable physical 70 properties and resistance to scaling and cracking appear to be at a maximum. A preferred analysis of the alloy is about 2.80% carbon, about 3% aluminum, about 3% silicon, about 3% chromium, and about .17% vanadium. 75

The alloy is well adapted for nitriding, and for certain purposes where a hard wear-resisting surface is desired, it is advisable to nitride the alloy. Any of the usual nitriding processes may be employed for this purpose.

It is preferred to form the alloy by melting in a crucible. It may, however, be made by any of the common methods of making cast iron, but an inferior product results. In carrying out the preferred crucible melting method, a pure iron containing carbon, but containing only small amounts of impurities such as sulphur, phosphorous and manganese, is melted in the crucible. It is preferred to use as the iron forming the base of the alloy, the metal known commercially as "washed metal", since this washed metal is substantially free from impurities and contains practically only iron and carbon. Less 85 satisfactory results may be obtained, however, by using other types of iron as the base metal. The necessary amounts of aluminum, silicon, chromium and vanadium to produce an alloy having the analyses above stated is added to 90 100

the washed metal, and the melting is controlled so as to give a resulting carbon content of 2.5 to 3.5%. It is preferred that the ferrous base, for example washed metal, contain not over .04% of phosphorus or sulphur, and not over 20% of manganese.

I have described in detail one method of producing my alloy. It is to be understood, however, that the alloy may be produced by other methods and that the alloy is not limited by the analysis given in the specific embodiment, but may be varied within the scope of the following claims.

I claim:

15 1. A ferrous alloy resistant to scaling and warping at high temperatures, and containing about 2.5% to 3.5% carbon, about 2.0% to 3.5% aluminum, about 2.0% to 3.5% silicon, about 2.0% to 3.5% chromium, and about 20 .10% to .50% vanadium, the balance being substantially iron.

25 2. A ferrous alloy resistant to scaling and warping at high temperatures, and containing about 2.5% to 3.5% carbon, about 2.0% to 3.5% aluminum, 2.0% to 3.5% silicon, about 2.0% to 3.5% chromium, and about .10% to .25% vanadium, the balance being substantially iron.

30 3. A ferrous alloy resistant to scaling and warping at high temperatures, and containing about 3.0% carbon, about 3.0% aluminum, about 3.0% silicon, about 3.0% chromium, and about .10% to .50% vanadium, the balance being substantially iron.

35 In testimony whereof I have hereunto set my hand.

RALPH L. BINNEY.